

hair  
hydraulic cement  
Plaster Paris

# UNITED STATES PATENT OFFICE.

E. H. ASHCROFT, OF LYNN, MASSACHUSETTS.

## IMPROVED NON-CONDUCTING COVERING FOR STEAM BOILERS, PIPES, &c.

Specification forming part of Letters Patent No. 59,338, dated November 6, 1866.

*To all whom it may concern:*

Be it known that I, EDWARD H. ASHCROFT, of the city of Lynn, county of Essex, in the Commonwealth of Massachusetts, have invented a new and Improved Non-Conducting Covering for Steam Boilers, Pipes, &c.; and I do hereby declare the following to be a true and exact description of the same.

The nature of my invention consists in providing a cheap and durable substitute for the hair or wool felting at present used as a covering for steam boilers, pipes, &c., acting as a non-conductor, economizing heat, preventing condensation of steam, accidents from fire, &c.

To enable those skilled in the art to make and use my invention, I will proceed to describe it.

The necessity of a non-conducting substance is too well known to need any further reference, and its extensive use on steam-vessels makes it an object to get a good and cheap material, the ordinary felting being expensive, and soon

becomes destroyed by the high degree of heat generated by the boilers. I therefore take ordinary hair, such as is used in mortars, and mix it either with hydraulic cement, lime and hydraulic cement, or plaster-of-paris, as follows: hair and hydraulic cement; hair, hydraulic cement, and plaster-of-paris; hair and cement of any kind, either of which can be applied as a covering (making a mortar) directly upon boilers or pipes. A coating of hair may be laid on and the cement poured upon it, so as to cover it entirely.

Having thus described my invention, what I claim as new, and desire to secure by Letters Patent of the United States, is—

A non-conducting covering for steam boilers, pipes, &c., composed of the materials above named, and applied as described.

E. H. ASHCROFT.

Witnesses:

JOHN P. WOODBURY,  
A. J. CHAN.